

## UNITED STATES PATENT OFFICE.

RENÉ BAURET, OF PARIS, FRANCE, ASSIGNOR TO LA SOCIETE: USINES METALLURGIQUES DE LA BASSE-LOIRE, OF PARIS, FRANCE, SIEGE SOCIAL.

## PROCESS FOR THE PRODUCTION OF BASIC STEEL.

No Drawing.

Application filed August 11, 1921. Serial No. 491,527.

*To all whom it may concern:*

Be it known that I, RENÉ BAURET, citizen of the Republic of France, and resident of Paris, Seine, France (post-office address 26<sup>bis</sup> 5 rue Alphonse de Neuville), Paris, have invented a new and useful Process for the Production of Basic Steel, which improvements are fully set forth in the following specification.

10 The present invention relates to a process for the production of basic steel, and is an improvement in or modification of the invention described and claimed in the specification of the co-pending application for 15 United States Patent Serial 468,762 herein-after referred to as the main patent.

In said main patent there has been described and claimed a process for the production of basic steel by the treatment in 20 the converter of grey pig iron with a silicon content above the normal, which could hitherto only be treated wastefully if at all, which consists in preparing in or introducing into the converter before the pig iron, 25 or the bulk of the pig iron is added, a liquid bath comprising oxides and lime adapted to oxidize the silicon of the pig iron immediately.

According to the present invention the 30 conversion process set forth in the main patent is utilized, for the production in a basic converter of hard steels, or semihard steels with a high carbon content, and totally dephosphorized, without it being necessary to 35 add to the metal, spiegeleisen, pig-iron or other re-carburizing agents.

It has been found, in carrying out the second phase of the operation according to the process forming the object of the main patent 40 in the presence of a calcareous slag rich in oxides of iron, that the newly charged pig-iron is dephosphorized very rapidly. This dephosphorization may be realized in practice before the carbon is entirely oxidized, so that by taking precautions to regulate the proportions of pig-iron added in each phase, it is easy to obtain steels, the analyses of which show a content of 0.50 45 and 0.60% carbon, with a content of 0.05% phosphorus. It has been found in practice that for charges of pig-iron exceeding 70%, (the normal charge of the usual processes.) the pressure of the blast does not exceed the pressure attained in ordinary operations,

this being in consequence of the very great 55 fluidity of the bath produced in the second operation. On the other hand, projections are entirely eliminated, and nothing prevents the filling of the converter to the maximum limit. It thus becomes possible in 60 practice to increase the yield in certain apparatus by at least 70%, this figure being liable to variation according to the shape of the converters.

An economic advantage is thus obtained 65 which is very important in the manufacture of hard steels or semi-hard steels with high carbon content and totally dephosphorized.

What I claim and desire to secure by Letters Patent is:—

1. The process for the production in a basic converter of hard steels with a high carbon content and practically dephosphorized, which consists in preparing in the converter before the pig iron is added a liquid bath comprising lime and oxides adapted to dephosphorize the pig iron very rapidly. 75

2. The process for the production in a basic converter of hard steels with a high carbon content and practically dephosphorized, which consists in preparing in the converter before the pig iron is added a liquid bath comprising lime and oxides of iron adapted to dephosphorize the pig iron very rapidly. 80

3. The process for the production in a basic converter of hard steels with a high carbon content and practically dephosphorized, which consists in preparing in the converter a liquid bath comprising lime and oxides of iron adapted to dephosphorize the pig iron very rapidly, and adding a predetermined amount of pig iron. 85 90

4. The process for the production in a basic converter of hard steels with a high carbon content and practically dephosphorized, which consists in preparing in the converter a predetermined quantity of a liquid bath comprising lime and oxides of iron adapted to dephosphorize the pig iron very rapidly, and introducing an abnormal charge of pig iron. 95 100

5. The process for the production in a basic converter of hard steels with a high carbon content and practically dephosphorized, which consists in preparing in the converter a liquid bath comprising lime and oxides of iron adapted to dephosphorize the 105

pig iron very rapidly, and filling the converter to the maximum limit with pig iron.

6. The process for the production in a basic converter of hard steels with a high carbon content and practically dephosphorized, which consists in preparing in the converter a predetermined quantity of a liquid bath comprising lime and oxides of iron adapted to dephosphorize the pig iron very

rapidly and filling the converter to the maximum limit with pig iron.

In testimony whereof I have signed this specification in the presence of two subscribing witnesses.

RENÉ BAURET.

Witnesses:

J. LEE MURPHY,

FERNAND DUFOUR.